

# UNITED STATES PATENT OFFICE.

WILLIAM H. BUELL, OF NEW HAVEN, CONNECTICUT, ASSIGNOR TO WINCHESTER REPEATING ARMS COMPANY, OF NEW HAVEN, CONNECTICUT, A CORPORATION OF CONNECTICUT.

## PRIMING CHARGE.

1,106,343.

Specification of Letters Patent.

Patented Aug. 4, 1914.

No Drawing.

Application filed October 21, 1913. Serial No. 796,441.

To all whom it may concern:

Be it known that I, WILLIAM H. BUELL, a citizen of the United States, residing at New Haven, in the county of New Haven, State of Connecticut, have invented a new and useful Improvement in Priming Charges; and I do hereby declare the following to be a full, clear, and exact description thereof.

10 My invention relates to a priming charge for use in igniting explosives, which is of especial utility in igniting the various smokeless and black powders when used in center fire and rim fire ammunition.

15 The purpose of my invention is to produce a priming charge which is particularly suited for use with powders as now employed in firearms, and particularly small arms, such charge producing an explosion of not too great local pressure, and of sufficient heat, and leaving substantially no harmful residues.

According to my invention I produce a priming charge by mixing intimately a detonating salt of hydrazoic acid with a suitable nitrated organic body. For instance, I 25 may add 3 parts by weight of nitrocellulose (preferably high nitrogen insoluble) to 1 part of lead hydrazoate, and mix the same to produce a substantially homogeneous product. While the detonating salts of hydrazoic acid are to *brisant* for use alone in firearms, and especially in small arms, the mixture above described will be found suitable for such use, the local pressure of the 30 explosion being reduced, and its heat increased. Substantially no residue is left which may injure the shell or the bore of the arm. While I prefer to use the lead salt, I may use other detonating salts of hydrazoic acid, for instance the silver salt; I may even use the mercury salt, although this salt 40 does not give all the contemplated advantages, as it leaves a residue which is apt to form a harmful amalgam with the metal of the shell.

In place of the nitrocellulose I may employ some other suitable nitrated organic body such for instance, as nitrated starch, the aromatic nitro compounds as trinitrotoluene; the nitro derivatives of carbamid or urea as nitrourea; the aromatic diazo salts as diazobenzene nitrate; and the aromatic diazoamido compounds as diazoamido benzene. While the proportions most suitable 50 for the mixture may differ with various sub-

stances, and also with various powders in connection with which the mixture is to be used, they are easily determined by any one skilled in the art.

I desire it to be understood that it is possible that some nitrated organic bodies, in combination with a detonating salt of hydrazoic acid, may not produce a primer having the explosive qualities above described, and that I therefore include in my invention the use of such bodies only as will in such combination produce such a primer.

It is also to be understood that the term "detonating salt" of hydrazoic acid as used in the art, and by me in this specification, refers only to a salt of the heavy metals, and does not include salts of the alkali metals, although such salts may have slight detonating properties under certain abnormal conditions.

The mixtures above specifically referred to constitute a fine white or light colored mass which may be moistened with a gum solution and then introduced into the primer cups, where it is seated under heavy pressure, and may then, if desired, be covered with paper or foil, or by a thin film of collodion. An anvil of any suitable construction may then be inserted into the cups. When the primer is to be used in rim fire ammunition it is preferably given the treatment with the gum solution and then driven into the annular rim of the cartridge shell by centrifugal force. It may then be covered by collodion.

The primer mixtures described in the above specific examples are homogeneous in character and of the proper igniting quality, so that a hot and uniform flame is produced without excess of local pressure and with a minimum of harmful residue or none at all. The flame produced has the proper velocity and intensity to ignite the powder charge before imparting any appreciable motion to it before ignition, and thus effects an explosion having the maximum pressure near the breech of the gun, and not one which is delayed until the charge nears the muzzle, the portion of the barrel least adapted to withstand bursting pressure.

While I may add other substances to my priming mixture, I prefer not to do so. Thus, chlorate of potash, or some other oxidizing compound, such as the perchlorates, nitrates and peroxides of barium, potassium,

- etc., may be added to the mixture, or in part substituted for certain ingredients, but their presence is usually undesirable owing to the production of an increased local pressure.
5. The subject matter of my invention must not be confused with detonators, nor with priming charges which are not suitable for use in firearms. To make a priming charge suitable for use in firearms it must not be
- 10 too violent in action, but must, on the other hand, be capable of being exploded by the action of the firing pin or other firing mechanism striking against the casing which contains the charge.
- 15 When I refer in my claims to a casing I mean to include in such term any container which is suitable for the purpose indicated, namely to permit the charge to be acted on by the firing mechanism.
- 20 I claim:
1. As an article of manufacture a casing suitable for use in connection with fire-arms, and a charge therein, said charge containing a mixture of a detonating salt of hydrazoic acid and a nitrated organic body, substantially as and for the purpose described.
  2. As an article of manufacture a casing suitable for use in connection with fire-arms, and a charge therein, said charge containing a mixture of a detonating salt of hydrazoic acid and a nitrated carbohydrate, substantially as and for the purpose described.

3. As an article of manufacture a casing suitable for use in connection with fire-arms, and a charge therein, said charge containing 35 a mixture of a detonating salt of hydrazoic acid and nitrocellulose, substantially as and for the purpose described.

4. As an article of manufacture a casing suitable for use in connection with fire-arms, 40 and a charge therein, said charge containing a mixture of lead hydrazoate and a nitrated organic body, substantially as and for the purpose described.

5. As an article of manufacture a casing 45 suitable for use in connection with fire-arms, and a charge therein, said charge containing a mixture of lead hydrazoate and a nitrated carbohydrate, substantially as and for the purpose described.

6. As an article of manufacture a casing suitable for use in connection with fire-arms, and a charge therein, said charge containing a mixture of lead hydrazoate and nitrocellulose, substantially as and for the purpose 55 described.

In testimony whereof I have hereunto set my hand in the presence of two subscribing witnesses.

WILLIAM H. BUELL.

Witnesses:

FRITZ ZIEGLER, Jr.  
JOHN A. FERGUSON.